

1,291,396

## UNITED STATES PATENT OFFICE.

SAMUEL BUTTERMAN, OF MADISON, WISCONSIN, ASSIGNOR TO UNITED STATES OF AMERICA.

## PROCESS OF MANUFACTURING WATERPROOF ADHESIVES.

1,291,396.

Specification of Letters Patent.

Patented Jan. 14, 1919.

No Drawing.

Application filed August 3, 1918. Serial No. 248,168.

106-78

*To all whom it may concern:*

Be it known that I, SAMUEL BUTTERMAN, a citizen of the United States, residing at Madison, in the county of Dane and State of Wisconsin, have invented a new and useful Improvement in Processes of Manufacturing Waterproof Adhesives, of which the following is a specification.

My invention relates to the manufacture of waterproof adhesives which remain for relatively long periods without "setting," that is, remain in a workable condition. It is well known that in most waterproof adhesives as now prepared "setting" or gelation takes place in a short time, usually within one or two hours after the adhesive has been prepared.

One of the objects of my invention is to overcome the instability which is usual in the preparation of glues. An adhesive prepared in accordance with my invention will remain stable and in a workable condition for a long period.

In carrying out my invention, I use by weight approximately one (1) part casein, one and five tenths (1.5) to two and eight tenths (2.8) parts water, fifteen thousandths (.015) parts hydrocarbon oil, fifteen hundredths (.15) parts powdered, hydrated lime, depending on the purity of the lime, a lesser percentage being required when pure lime is used and a greater percentage when the lime is of inferior quality, mixed in ninety hundredths (.90) parts water and seventy hundredths (.70) silicate of soda.

To prepare an adhesive in accordance with my invention, the ingredients specified may be combined in the following manner: The oil is first mixed with the dry casein. This may be done by spraying the casein with oil. To the casein and oil the water specified is now added and the mixture is allowed to soak for about one-half hour. At the end of this period the mixture is rapidly agitated

and the water and lime are introduced. 45 After a few minutes the silicate of soda is added and the stirring is continued from twenty minutes to one half hour, until a smooth uniform texture free from lumps obtains. The adhesive is then ready for use. 50

As the function of the oil is a mechanical one, added for the purpose of allowing the dry casein to be handled without inconvenience and increasing the flexibility of the dry glue layer, I may use various kinds of 55 oil. I have found, however, that kerosene or paraffin oils give good results.

It should be noted that the proportions of the ingredients used by me are stated approximately and that I do not limit myself 60 to the proportions named as they may be varied considerably without affecting unfavorably the results obtained.

What I claim is:

1. A composition of matter comprising by 65 weight approximately one (1) part casein, two (2) parts water, fifteen thousandths (.015) parts oil, fifteen hundredths (.15) parts powdered, hydrated lime, mixed in ninety hundredths (.90) parts water, and 70 seventy hundredths (.70) parts silicate of soda.

2. The herein described method of preparing adhesive consisting of mixing by weight approximately one (1) part casein with fifteen thousandths (.015) parts oil, adding to this mixture between one and five tenths (1.5) and two and eight tenths (2.8) parts water, allowing this mixture to soak approximately one-half hour, then adding fifteen 80 hundredths (.15) parts powdered, hydrated lime, mixed in ninety hundredths (.90) parts water, and then adding to this mixture within a few minutes seventy hundredths (.70) parts silicate of soda. 85

In testimony whereof I have hereunto affixed my signature.

SAMUEL BUTTERMAN.